

## UNITED STATES PATENT OFFICE.

EDWARD D. FROHMAN, OF PITTSBURGH, PENNSYLVANIA.

## WASH FOR SAND CORES AND MOLDS FOR METAL FOUNDRY.

No Drawing.

Application filed November 16, 1925. Serial No. 69,513.

My improved wash is particularly adapted for steel castings but it may be used with advantage in making castings of other metals. The present practice is to use a wash made by mixing silica ( $SiO_2$ ) with molasses. In the use of a wash of this character frequently the material of the wash sticks to the metal when the same is poured, and it is difficult to clean the castings when removed from the mold. It is also difficult to finish a casting when such a wash has been used because of the formation of the iron-silicates on the surface of the casting, the finishing tools becoming quickly dulled on account of the hardness. This adds to the time and the labor required for turning out a finished casting.

The object which I have in view is the provision of a wash which will cause the casting to be readily cleansable and which will impart to the casting a soft alumina-alloy surface which is easily cut in the finishing operation.

For this purpose I have invented a new and improved wash characterized by the presence of bauxite or alumina-oxide ( $Al_2O_3$ ).

More particularly my wash is formed of a composition of bauxite and organic oil and a binder.

The organic oil is preferably a vegetable oil, and I have found satisfactory linseed oil or soya bean oil.

For a binder I have successfully used sulphite pitch, molasses or dextrose.

The proportions which I find to be advantageous are approximately one hundred pounds of bauxite, not more than three pounds of oil, and not more than three pounds of binder.

In preparing the wash I prefer to first mix the binder and oil together and then add the bauxite in small quantities together with sufficient water so that as it is stirred

a composition of putty like consistency is obtained. The wash composition may be packed and shipped in this form.

When the wash is to be gotten ready for use it is mixed with sufficient water to obtain a composition of paint like consistency which can be readily brushed or sprayed on the cores or molds.

If desired, of course, in making the original mixture sufficient water may be employed to obtain a paint like consistency instead of a putty like consistency, but where the wash-compound is prepared at a factory for shipment to the foundry, it is preferable to produce the putty like form, as it can be more advantageously barreled or otherwise packed for delivery.

The fusing point of bauxite or alumina-oxide is approximately 3200 degrees Fahr., while that of steel in proper molten form for pouring is approximately 2700 degrees Fahr. As a result the bauxite does not fuse in the presence of the molten steel and therefore there is no burning in of the materials of the wash in the steel of the casting.

When the casting is removed from the mold there is found deposited on the surface thereof a thin layer of bauxite which being relatively soft is easily and quickly removed by a sand blast or by the finishing tool.

What I desire to claim is:—

1. A wash compound for foundry cores and molds comprised of alumina-oxide, a binder and organic oil.

2. A wash compound for foundry cores and molds comprised of alumina-oxide, a binder and organic oil in substantially the proportions of three pounds each of the binder and the oil to one hundred pounds of alumina-oxide.

Signed at Pittsburgh, Pa., this 13th day of November, 1925.

EDWARD D. FROHMAN.